

## [54] MERCERIZING SOLUTIONS

[75] Inventors: **Hans-Jerg Kleiner**, Bad Soden, Taunus; **Karl-Heinz Schneider**, Kelkheim, Taunus; **Gerhart Schneider**, Schneidhain, Taunus, all of Germany

[73] Assignee: **Hoechst Aktiengesellschaft**, Frankfurt am Main, Germany

[22] Filed: June 21, 1973

[21] Appl. No.: 372,330

2,236,617 4/1941 Brandt ..... 8/127  
 2,403,038 7/1946 Aelony ..... 8/127  
 2,478,390 8/1949 Hanford et al. ..... 260/459  
 S325,654 4/1943 Volz ..... 8/127

Primary Examiner—Benjamin R. Padgett

Assistant Examiner—B. Hunt

Attorney, Agent, or Firm—Connolly and Hutz

## [57]

## ABSTRACT

Aqueous mercerizing solutions containing an alkali metal hydroxide and an alkali metal salt of a phosphinic acid of the formula



in which  $\text{R}_1$  is methyl or ethyl and  $\text{R}_2$  is an aliphatic hydrocarbon radical of 4 to 12 carbon atoms, and the use of these solutions for mercerizing cellulosic fibrous materials.

## [30] Foreign Application Priority Data

June 26, 1972 Germany ..... 2231147

[52] U.S. Cl. ..... 8/127; 8/125  
 [51] Int. Cl. ..... D06m 1/02  
 [58] Field of Search ..... 8/116 P, 127, 125

## [56] References Cited

## UNITED STATES PATENTS

1,980,342 11/1934 Kern ..... 8/127

4 Claims, 2 Drawing Figures



Shrinkage Rate  
mm/sec



FIG. 2

## MERCERIZING SOLUTIONS

The present invention relates to aqueous solutions containing alkaline agents and phosphinic acids for mercerizing purposes.

For the purpose of mercerizing and treating cellulosic fibers, especially cotton fibers and goods made therefrom, with lyes, alkali metal hydroxide solutions having a strength sufficient to meet certain requirements are allowed to act on the material. To accelerate this operation thus assuring a continuous and economical working process, it is necessary to have the material soaked with alkaline solution as quickly and uniformly as possible. To this effect, wetting agents are added to the solutions while making sure that these are readily soluble in the lye, bring about a maximum shrinkage rate of the cellulosic fiber within the shortest possible time and remain in solution even after the lyes have been stored for a prolonged period of time.

It is already known that alkyl sulfates, alkane sulfonates, alkyl-aryl sulfonates, lignin sulfonic acids, sulfated terpene derivatives, alkylated naphthalene sulfonic acids and analogous compounds can be used as wetting agents in mercerizing liquors. German Auslegeschrift No. 1,014,067 discloses the application of mixtures of such mono and polysulfonic acids or salts thereof in mercerizing baths. Those compounds have been obtained by sulfo-chlorination of aliphatic or cycloaliphatic hydrocarbons having 10 to 20 carbon atoms.

The wetting agents are generally combined with other adjuvants which disperse and keep in suspension the products which have been dissolved off the fiber during the mercerizing operation, for example cellulose degradation compounds or remaining sizes. At the same time, these adjuvants have a synergistic effect on the wetting power of the wetting agents which are known to be low-molecular-weight alcohols, for example isopropanol, butanols, alkanol-amines, glycols and derivatives thereof, polyglycols and other compounds disclosed, inter alia, in Lindner "Tenside, Textilhilfsmittel, Waschrohstoffe", vol. II, 1964, pages 1476 to 1478.

Wetting agents hitherto used for mercerizing liquors do not meet all the practical requirements at the same time. They either wet the fiber very rapidly while having to be used, however, in high concentrations or they are not stable in the alkaline solutions for a sufficiently long time, lose their effectiveness or precipitate. In many cases, moreover, their heavy foaming is troublesome.

This invention now relates to aqueous solutions for mercerizing and treating cellulosic fibers and goods made therefrom with lyes, which have an excellent wetting effect and a high stability and contain, in addition to about 10 to 400 g/l of sodium, potassium or lithium hydroxide or mixtures of these alkaline agents, as wetting agents, from 0.1 to 5 g/l of phosphinic acids of the general formula



in which  $R_1$  stands for a methyl or ethyl group and  $R_2$  for an aliphatic linear, branched or cyclic hydrocarbon radical having 4 to 12 carbon atoms, preferably 6 to 10 carbon atoms, in the form of their alkali metal salts as essential ingredients.

The phosphinic acids or the alkali metal salts thereof to be used as wetting agents according to the invention may be prepared according to various methods, for example by the known reaction of sodium salt of methane-phosphonic acid monoethyl ester with Grignard compounds (cf. K. A. Petrov et al., Z. obsc. Chim. 30 1964-8 (1960); C.A. 55, 6363b (1961). The process disclosed in French Patent No. 7,045,130 and German Offenlegungsschrift No. 2,100,779 is especially preferred, according to which dialkyl phosphinic acid alkyl esters of the general formula



in which  $R_1$  is alkyl of 2 to 22 carbon atoms and  $R_2$  and  $R_3$  each is alkyl of 1 to 22 carbon atoms, are prepared by an addition reaction of  $\alpha$ -olefins of 2 to 22 carbon atoms with phosphorous acid alkyl esters of the formula



in which  $R_2$  and  $R_3$  are defined as above. As phosphorous acid alkyl esters suitable for this reaction, there are mentioned, for example, methane-phosphorous acid methyl ester, methanephosphorous acid ethyl ester, octane-phosphorous acid ethyl ester. The salts or free acids thereof may be prepared from the dialkyl phosphinic acid esters by hydrolysis according to known methods, advantageously by an alkaline saponification. The solutions of the invention may, however, also be prepared using the dialkyl phosphinic acid esters or the free acids, thereof.

The phosphinic acids and the salts thereof to be used according to the invention are readily soluble in water and give limpid solutions. In an alkaline medium, they have such an excellent wetting power that they can be used in lower amounts than conventional wetting agents. The concentrations used in the mercerizing solutions are between 0.1 and 5 g/l, which means not only a very economical application of the compounds but also hardly any pollution of waste water. Furthermore, the phosphinic acids and the salts thereof do practically not foam in the alkaline solutions. They are preferably used for mercerizing liquors containing a high amount of about 150 to 300 g, preferably 200 to 250 g of sodium-, potassium- or lithium hydroxide or mixtures thereof per liter of liquor.

The known addition of lower alcohols, for example isopropanol or butanol, or of alkanol-amines, for example butyl-diethanol-amine, to the mercerizing solutions, may further improve the wetting power of the solutions.

The composition of the mercerizing solutions, for which the phosphinic acids or the salts thereof are used

according to the invention, is known; they generally contain 10 to 400 g of sodium-, potassium- or lithium hydroxide or mixtures thereof per liter of liquor and, where required, further usual adjuvants. The solutions are used at temperatures of from about 0° to 25°C. As 5 to further additives, see Lindner "Tenside, Textilhilfsmittel, Waschrohstoffe", vol. II, 1964, pages 1476 to 1478, and Ullmanns Encyclopadie der technischen Chemie, 3rd edition, vol. 17, 1966, pages 176 to 177.

By the way, it is not necessary at any circumstances 10 to convert the dialkyl phosphinic acid esters prepared according to the prior art indicated above into the corresponding acids or alkali salts to use them according to the invention. It is also possible to add the esters directly to the mercerizing solutions, since they are hydrolyzed in the alkaline liquor to yield the salts.

The mercerizing solutions of the invention are used in known manner for treating cellulosic fibers and goods made therefrom as well as textile material containing cellulosic fibers in addition to synthetic fibers. 20

For further illustration, the values of shrinkage and shrinkage rate are given diagrammatically by way of example in the accompanying drawings.

FIG. 1 shows the values of shrinkage as a function of time using liquors Nos. 1, 5 and 6. 25

FIG. 2 shows the corresponding values of shrinkage rate as a function of time.

The following Examples serve to illustrate the invention.

15 The good stability of the phosphinic acids used according to the invention even in lyes having an extremely high concentration of alkalis is demonstrated by the results obtained with

Liquors No. 7 and 7 (a): 330 g/l of sodium hydroxide and 2.5 g/l of methyl-hexyl-phosphinic acid.

20 Liquors Nos. 3 (a) and 7 (a) had the same composition as liquors Nos. 3 and 7 but had been allowed to stand for 24 hours prior to its use for the tests.

25 The test results are compiled in the following Table.

TABLE

| Time<br>sec. | shrinkage in<br>mm |     |     |     |    |     |    |    |    |    |    |    |    |    | shrinkage rate<br>in mm/sec. |    |    |    |  |  |  |  |
|--------------|--------------------|-----|-----|-----|----|-----|----|----|----|----|----|----|----|----|------------------------------|----|----|----|--|--|--|--|
|              | Liquor number      |     |     |     |    |     |    |    |    |    |    |    |    |    |                              |    |    |    |  |  |  |  |
|              | 1                  | 2   | 3   | 3a  | 4  | 5   | 6  | 7  | 7a | 1  | 2  | 3  | 3a | 4  | 5                            | 6  | 7  | 7a |  |  |  |  |
| 5            | 22                 | 13  | 58  | 57  | 3  | 47  | 4  | 25 | 20 | 22 | 13 | 58 | 57 | 3  | 47                           | 4  | 25 | 20 |  |  |  |  |
| 10           | 74                 | 50  | 92  | 88  | 36 | 90  | 14 | 55 | 50 | 52 | 37 | 34 | 31 | 33 | 43                           | 10 | 30 | 30 |  |  |  |  |
| 20           | 119                | 90  | 98  | 98  | 71 | 97  | 34 | 73 | 70 | 45 | 40 | 6  | 10 | 35 | 7                            | 20 | 18 | 20 |  |  |  |  |
| 30           | 126                | 95  | 99  | 99  | 75 | 99  | 51 | 76 | 76 | 7  | 5  | 1  | 1  | 4  | 2                            | 17 | 3  | 6  |  |  |  |  |
| 45           | 129                | 98  | 99  | 100 | 78 | 101 | 64 | 78 | 78 | 3  | 3  | 0  | 1  | 3  | 2                            | 13 | 2  | 2  |  |  |  |  |
| 60           | 130                | 99  | 100 | 100 | 80 | 102 | 75 | 79 | 79 | 1  | 1  | 1  | 0  | 2  | 1                            | 11 | 1  | 1  |  |  |  |  |
| 75           | 130                | 100 | 101 | 101 | 81 | 102 | 80 | 79 | 79 | 0  | 1  | 1  | 1  | 1  | 0                            | 5  | 0  | 1  |  |  |  |  |
| 90           | 132                | 101 | 101 | 101 | 82 | 103 | 84 | 80 | 80 | 2  | 1  | 0  | 0  | 1  | 1                            | 4  | 1  | 1  |  |  |  |  |

## EXAMPLES

Since the wetting power of strongly alkaline liquors cannot be measured using conventional devices according to German Industrial Standards (DIN) 53 901, the following tests were carried out using, as a measure for the wetting power of a mercerizing liquor, the shrinkage of cotton in this liquor. For this purpose, a test device suitable for measuring mercerizing liquors according to Hintzmann was used. This device is described in detail in "Melland Textilberichte" (1968), No. 3, pages 311 to 315 and No. 4, pages 450 to 456. This device was operated at 20°C with an amount of 250 cc. under a charge of 33 grams. Measuring was performed on cotton hanks (70/2-fold) having a length of 27.4 cm. Shrinkage was measured after a period of action of the liquor of 5, 10, 20, 30, 45, 60, 75 and 90 seconds. The shrinkage rate in mm/sec. was calculated from the shrinkage values obtained in mm.

50 All the tested mercerizing liquors contained 220 g of sodium hydroxide per liter and, in addition, the following wetting agents and adjuvants:

The results convincingly demonstrate the advantage of the phosphinic acids and the alkali metal salts thereof to be used according to the invention. The results measured on liquors Nos. 3 and 3 (a) show an unaltered wetting power of the mercerizing solutions of the invention even after a storage time of 24 hours.

We claim:

55 1. An aqueous mercerizing solution essentially consisting of about 10 to 400 g/l of sodium, potassium or lithium hydroxide or a mixture thereof, and 0.1 to 5 g/l of a phosphinic acid of the formula



60 65 in which  $R_1$  stands for a methyl or ethyl group and  $R_2$  stands for an aliphatic linear, branched or cyclic hydrocarbon radical having 4 to 12 carbon atoms, in the form of its alkali metal salt.

5

2. An aqueous mercerizing solution as claimed in claim 1 having a content of 0.1 to 5 g/l of methyl-octyl phosphinic acid in the form of its alkali metal salt.

3. An aqueous mercerizing solution as claimed in claim 1 having a content of 0.1 to 5 g/l of methyl-hexyl phosphinic acid in the form of its alkali metal salt.

4. A process for treating with lyes and mercerizing cellulosic fibrous material, which comprises treating the fibrous material with an aqueous alkaline mercerizing solution essentially consisting of about 10 to 400 g/l of sodium, potassium or lithium hydroxide and as a wetting agent 0.1 to 5 g/l of a phosphinic acid of the formula



in which  $R_1$  stands for a methyl or ethyl group and  $R_2$  for an aliphatic linear, branched or cyclic hydrocarbon radical having 4 to 12 carbon atoms, preferably 6 to 10 carbon atoms, in the form of its alkali salt.

21

25

30

15

65